

## UNITED STATES PATENT OFFICE

2,291,052

## PRINTING CELLULOSE ACETATE

Charles Franklin Miller, Wilmington, Del., assignor to E. I. du Pont de Nemours & Company, Wilmington, Del., a corporation of Delaware

No Drawing. Application July 9, 1940.  
Serial No. 344,494

7 Claims.

(Cl. 8—63)

This invention relates to a process for printing cellulose esters with acid and direct dye-stuffs.

It has been proposed to use thiocyanates in the printing of cellulose ester fabrics but we have found that, when such agents are used in printing compositions with acid or direct dye-stuffs, they do not produce satisfactory prints. The unsatisfactory result is most frequently indicated by weakness of the printing.

It is an object of my invention to improve the printing of acid and direct colors on cellulose acetate.

The objects of my invention are accomplished, generally speaking, by printing cellulose acetate with acid or direct color with an aqueous medium containing the color, a hydrotropically active agent of a particular class, and zinc thiocyanate. Although I do not wish to be limited to any particular theory of operation, it appears that, by reducing the state of aggregation of the acid or direct color in an aqueous medium containing zinc thiocyanate, and applying the medium to cellulose acetate, there is produced a greatly improved printing. It is my surprising discovery that thiocyanates in general do not produce the invention and that hydrotropical agents in general do not produce the invention, but that the invention is produced by the combination of zinc thiocyanates with hydrotropical agents of the following classes: urea, thiourea, soluble metal salts of aliphatic sulfuric or sulfonic acids of one to twelve carbon atoms, soluble metal salts of aromatic sulfonic acids which may contain hydroxy, nitro, or halogen substituents in the nucleus, soluble metal salts of aryl, alkyl or aralkyl thioglycolic acid. The alkali earth thiocyanates, the organic thiocyanates, and the ammonium, iron, cadmium, tin, and manganese thiocyanates all have objectionable features.

Among the hydrotropical compounds the following are named as exemplary: sodium ethyl butyl phthalate, sodium N. octyl sulfate, sodium N. propyl sulfate, N. isopropyl sulfate, sodium N. hexyl phthalate, sodium tetraline sulfonate, sodium para phenol sulfonate, potassium alpha naphthalene sulfonate, sodium benzyl thioglycolate, sodium methyl adipate, sodium benzyl succinate, sodium isobutyl sulfate, thio urea, sodium N-butyl sulfonate, zinc p-toluene sulfonate.

Among the advantages that are gained by my invention are freedom from gas fume fading, greater freedom from "crocking" and sublima-

tion on steaming, greater range of colors and greater choice of colors and greater strength.

The following examples illustrate the invention but do not limit it:

|    |                                  |                 |
|----|----------------------------------|-----------------|
| 5  | Example I                        | Parts by weight |
|    | Direct color dyestuff—C. I. #814 | 3.00            |
| 10 | Urea                             | 15.00           |
|    | Zinc thiocyanate                 | 10.00           |
| 15 | Water                            | 12.00           |
|    | Thickening—50% British gum       | 60.00           |
|    |                                  | 100.00          |

15 The above described printing paste is printed on acetate process rayon, dried, steamed 45 minutes in a "cottage steamer," soaped lightly and dried giving a bright, even yellow design which is many times stronger than can be obtained with the above dyestuff without the assistants or with the assistants singly.

|    |                                |                 |
|----|--------------------------------|-----------------|
| 20 | Example II                     | Parts by weight |
|    | Acid color dyestuff—C. I. #430 | 3.00            |
| 25 | Sodium para toluene sulfonate  | 10.00           |
|    | Zinc thiocyanate               | 10.00           |
|    | Water                          | 17.00           |
|    | 50% British gum                | 60.00           |
|    |                                | 100.00          |

30 The described printing paste is printed and finished as in Example I giving a clear, brilliant red design.

|    |                                  |                 |
|----|----------------------------------|-----------------|
| 35 | Example III                      | Parts by weight |
|    | Direct color dyestuff—C. I. #319 | 3.00            |
| 40 | Sodium N. butyl sulfate          | 5.00            |
|    | Zinc thiocyanate                 | 10.00           |
|    | Water                            | 22.00           |
|    | 50% British gum                  | 60.00           |
|    |                                  | 100.00          |

45 The described printing paste was printed and finished as in Example I, giving a brilliant violet design.

|    |                                     |                 |
|----|-------------------------------------|-----------------|
| 50 | Example IV                          | Parts by weight |
|    | Acid color dyestuff—C. I. #216      | 3.00            |
|    | Potassium methyl pentanol phthalate | 5.00            |
|    | Zinc thiocyanate                    | 10.00           |
|    | Water                               | 22.00           |
|    | 50% British gum                     | 60.00           |
|    |                                     | 100.00          |

The described printing paste was printed and finished as in Example I, giving a bright orange design.

The following colors, when treated in the manner described, also illustrate the invention:

- Ex. 5.—Direct color dyestuff—C. I. # 813
- Ex. 6.—Direct color dyestuff—C. I. # 561
- Ex. 7.—Direct color dyestuff—C. I. # 581
- Ex. 8.—Direct color dyestuff—C. I. # 812
- Ex. 9.—Acid color dyestuff —C. I. # 307
- Ex. 10.—Acid color dyestuff —C. I. # 289
- Ex. 11.—Acid color dyestuff —C. I. # 666
- Ex. 12.—Acid color dyestuff —C. I. # 1080
- Ex. 13.—Acid color dyestuff —C. I. # 1088
- Ex. 14.—Direct color dyestuff—C. I. # 620
- Ex. 15.—Direct color dyestuff—C. I. # 816
- Ex. 16.—Acid color dyestuff —C. I. # 670

As many apparently widely different embodiments of this invention may be made without departing from the spirit and scope thereof, it is to be understood that I do not limit myself to the specific embodiments thereof except as defined in the appended claims.

I claim:

- 1. The process of printing cellulose acetate with acid and direct dyestuffs which comprises reducing the state of aggregation of the dyestuff in an aqueous medium containing zinc thiocyanate, and a hydrotropical agent from the class consisting of urea, thiourea, soluble metal salts of aliphatic sulfuric acids having up to twelve carbon atoms, soluble metal salts of aliphatic sulfonic acids having up to twelve carbon atoms, soluble metal salts of aromatic sulfonic acids, soluble metal salts of aryl, alkyl, and aralkyl thioglycollic acids, and soluble metal salts of alkyl, aryl and aralkyl dicarboxylic acid mono-esters and printing the cellulose acetate with the said aqueous medium containing the dyestuff. 30

- 2. The process of printing cellulose acetate with acid and direct dyestuff which comprises incorporating the dyestuff in an aqueous medium containing zinc thiocyanate and a hydrotropical agent from a class consisting of urea, thiourea, soluble metal salts of aliphatic sulfuric acids having up to twelve carbon atoms, soluble metal salts of aliphatic sulfonic acids having up to twelve carbon atoms, soluble metal salts of aromatic sulfonic acids, soluble metal salts of aryl, alkyl, and aralkyl thioglycollic acids, and soluble metal salts of alkyl, aryl, and aralkyl dicarboxylic acid mono-esters. 5
- 3. The process of printing cellulose acetate with acid and direct dyestuffs which comprises incorporating the dyestuff in an aqueous medium containing zinc thiocyanate and a compound of the class consisting of soluble metal salts of alkyl, aryl, and aralkyl dicarboxylic acid mono-esters. 15
- 4. The process of printing cellulose acetate with acid and direct dyestuffs which comprises incorporating the dyestuff in an aqueous medium containing zinc thiocyanate and a soluble metal salt of a phthalic acid mono-ester. 20
- 5. The process of printing cellulose acetate with acid and direct dyestuffs which comprises incorporating the dyestuff in an aqueous medium containing zinc thiocyanate and sodium ethyl butyl phthalate. 25
- 6. The process of printing cellulose acetate with acid and direct dyestuffs which comprises incorporating the dyestuff in an aqueous medium containing zinc thiocyanate and sodium-N-hexyl phthalate. 30
- 7. The process of printing cellulose acetate with acid and direct dyestuffs which comprises incorporating the dyestuff in an aqueous medium containing zinc thiocyanate and potassium methyl pentanol phthalate. 35

40

CHARLES FRANKLIN MILLER.